

Oct. 30, 1951

J. D. KENDALL ET AL

2,573,027

PHOTOGRAPHIC ELEMENT AND PROCESS UTILIZING ANTIBRONZING AGENTS

Filed Nov. 8, 1945

*Fig. 1.*



*Fig. 2.*



*Fig. 3.*



INVENTORS

*John David Kendall and  
Douglas James Fry*

BY *Stevens, Davis, Miller and Mosher*  
ATTORNEYS

## UNITED STATES PATENT OFFICE

2,573,027

PHOTOGRAPHIC ELEMENT AND PROCESS  
UTILIZING ANTIBRONZING AGENTSJohn David Kendall and Douglas James Fry,  
Ilford, England, assignors to Ilford Limited,  
Ilford, Essex, England, a British companyApplication November 8, 1945, Serial No. 627,518  
In Great Britain November 13, 1944

16 Claims. (Cl. 95-7)

**1**

This invention relates to compounds which serve as improvers for photographic silver halide emulsions and particularly to compounds which, when included in the emulsion layer, or in another layer present in the photographic material, or when added to the developer, fixer or other processing bath applied to the photographic material, improve the quality of the developed photographic images obtained.

In the production of photographic images in silver halide emulsions, and particularly in the case of emulsions in which the silver halide is predominantly silver chloride, the maximum image density obtainable is not always so great as may be desired. Moreover, the common practice of hot-glazing photographic prints tends to affect adversely the image colour, giving a poor quality black having a "bronzed" appearance, and also reduces the effective maximum density obtainable in the image.

It has now been discovered that this bronzing effect may be reduced or eliminated and the maximum density obtainable may be increased by bringing into contact with the photographic emulsion a member of a certain class of heterocyclic nitrogen compounds, and according to this invention, therefore, a method of improving photographic silver halide emulsions in regard to the quality of the images developed therein comprises including in the emulsion, or in another layer of a photographic element containing such emulsion, or in a developing, fixing or other processing bath with which the photographic element is treated, a heterocyclic compound containing two nitrogen atoms in the ring and one, two or three sulphur atoms attached to carbon atoms which are in  $\alpha$ -positions to the nitrogen atoms (but excluding the case where a single sulphur atom is present and attached to a carbon atom which is  $\alpha$  to both nitrogen atoms), the nitrogen atoms being unsubstituted. Such compounds contain at least one sulphur atom attached to a carbon atom  $\alpha$  to a nitrogen atom on one side and an atom of an element different from nitrogen on the other side. Typical forms of compound are those having the groupings:

**2**

as part of the heterocyclic ring. The compounds of the type



5 where there is a single sulphur atom between two nitrogens, are not included since in this case the carbon atom to which the sulphur is attached is  $\alpha$  to both nitrogen atoms.

10 The following are illustrative classes of compounds which may be employed.

A. Compounds which have one of the following tautomeric forms:



15 20 where X is an oxygen atom or a sulphur atom and Y is an oxygen atom, a sulphur atom or an imino group. Examples of this class are:

2:5-dimercapto-1:3:4-thiodiazole  
2-mercaptop-5-amino-1:3:4-thiodiazole

25 B. Compounds which have one of the following tautomeric forms:



30 35 where D represents the carbon atoms completing a six-membered ring and may include a fused benzene ring, and Y is oxygen, sulphur, or an imino group. Examples of this class of compound are:

40 1-mercaptop-4-hydroxy-phthalazine  
1:4-dimercapto-phthalazine

C. Compounds of the general formula:



45 50 where D and Y have the same significance as in B above. Examples of this type of compound are:

55 2-hydroxy-4-mercaptop-pyrimidine  
2:4-dimercapto pyrimidine  
2:4-dimercapto quinazoline

## 3

This class of compound includes compounds of the general formula:



where Y has the same significance as given above. An example of this type of compound is trithio barbituric acid.

It will be understood that all these compounds may exist in tautomeric forms, the



grouping tautomerising to



and that any of the tautomeric forms may be employed in this invention. The common names given to the compounds sometimes refer more accurately to the alternative tautomeric formulae. Some of the free compounds are somewhat unstable and these compounds, and indeed any of the compounds, may be used in the form of their alkali metal or ammonium salts.

As already indicated these compounds may be included in the silver halide photographic emulsion or in another layer of the photographic element, preferably coated adjacent to such emulsion layer, for example in a sub-coat layer or in a super-coat layer. The optimum quantity of compound to be employed will always be small, but will depend on the particular substance selected. In general it is found that for incorporation in an emulsion, sub-coat or super-coat, a proportion of 1 part of the compound in 1000 to 100,000 of the emulsion, super-coat or sub-coat solution is generally suitable, while for incorporation in a developer, fixer or other processing bath, e. g. a glazing solution, the optimum quantity may be, for example, between 1 part in 3000 to 1 part in 300,000 parts of the processing solution. Frequently even lower concentrations than those given above have some effect and, though it may be uneconomic in being a waste of material, even higher concentrations may be employed.

More than one compound of the type defined may be used if desired, and the compound or compounds may be included in more than one position, e. g. in super-coat and developing solution, or in both developing and fixing solutions.

In general the compounds will be applied to the photographic emulsion before reaching the final stage of drying the developed image, but they may be applied with advantage to already dried prints where it is desired to subject the latter to hot-glazing.

The following examples illustrate the invention:

## Example 1

To a silver chloride photographic emulsion of the type known as a "vigorous gaslight" emulsion (A) and to a silver bromide emulsion of the type used for vigorous bromide printing paper (B), was added 21 cc. of a 0.5% solution in ethyl alcohol of 2:5-dimercapto-1:3:4-thiodiazole per litre of emulsion. The emulsions were coated on paper. Comparative tests (controls) were made with the same emulsions not containing the said compound. Test strips of the papers thus ob-

## 4

tained were exposed, developed, fixed, washed and hot-glazed shortly after coating, and similar test strips were exposed, developed, fixed, washed and hot-glazed after the paper had been kept for some hours in a warm moist atmosphere (i. e. "incubated"). The test strips were examined visually and sensitometrically and gave the following results:

| Emulsion (A or B)                                        | Degree of bronzing after hot-glazing  | Maximum density of samples tested shortly after coating | Maximum density of "incubated" samples |
|----------------------------------------------------------|---------------------------------------|---------------------------------------------------------|----------------------------------------|
| Control A.....<br>Tests A containing the above compound. | considerable...<br>very much reduced. | 1.72<br>2.10                                            | 1.69<br>2.00                           |
| Control B.....<br>Tests B containing the above compound. | considerable...<br>much reduced.      | 1.64<br>1.97                                            | 1.90<br>2.03                           |

## Example 2

To a gelatin super-coat solution was added 22 cc. of a 0.5% solution in ethyl alcohol of 2:5-dimercapto-1:3:4-thiodiazole per litre of the super-coat solution. This solution was coated on the surface of layers of the emulsions referred to in Example 1 carried on paper supports. Control tests were made with super-coats of similar composition but not containing the said compound. Test strips were prepared as in Example 1 and the following results were obtained:

| Emulsion (A or B)              | Degree of bronzing after hot-glazing | Maximum density of samples tested shortly after coating | Maximum density of "incubated" samples |
|--------------------------------|--------------------------------------|---------------------------------------------------------|----------------------------------------|
| Control A.....<br>Tests A..... | considerable...<br>much reduced.     | 1.72<br>2.06                                            | 1.69<br>2.02                           |
| Control B.....<br>Tests B..... | considerable...<br>much reduced.     | 1.64<br>1.98                                            | 1.90<br>2.02                           |

## Example 3

The procedure of Example 2 was followed with the following compounds in the quantities indicated:

Cc.

- (a) 1-mercaptop-4-hydroxy phthalazine..... 22
- (b) 1:4-dimercapto phthalazine..... 45
- (c) 2-hydroxy-4-mercaptop-pyrimidine..... 45
- (d) 2:4-dimercapto pyrimidine..... 45
- (e) 2:4-dimercapto quinazoline..... 45
- (f) Trithio barbituric acid..... 22

In all cases the control samples showed considerable bronzing on hot-glazing, whereas in the test samples the degree of bronzing was much reduced or entirely eliminated. The following table sets out the maximum density of the images obtained after hot-glazing shortly after coating:

| Compound       | Emulsion A | Emulsion B |
|----------------|------------|------------|
| Control a..... | 1.56       | 1.71       |
| Control b..... | 1.97       | 1.79       |
| Control c..... | 1.67       | 1.76       |
| Control d..... | 1.92       | 1.99       |
| Control e..... | 1.56       | 1.56       |
| Control f..... | 2.03       | 2.04       |
| Control g..... | 1.56       | 1.55       |
| Control h..... | 2.03       | 2.03       |
| Control i..... | 1.67       | 1.76       |
| Control j..... | 1.96       | 2.06       |
| Control k..... | 1.56       | 1.71       |
| Control l..... | 1.97       | 2.03       |

It will be seen that in all cases a substantial increase in the maximum density was obtained.

## 5

## Example 4

A 1:500 solution of 2:5-dimercapto-1:3:4-thiodiazole in N/25 sodium carbonate solution was prepared. This was added to a 20% acid hypo fixing bath at the rate of 75 cc. per litre. The fixing bath thus prepared was employed for fixing developed images in a normal "gaslight" printing paper (A) of which the silver halide of the emulsion was primarily silver chloride, and in a normal "bromide" printing paper (B) of which the silver halide of the emulsion was primarily silver bromide. Control tests were carried out at the same time with a similar fixing bath not containing the compound. The results obtained were as follows:

| Emulsion (A or B) | Degree of bronzing after hot-glazing | Maximum density of developed and fixed image |
|-------------------|--------------------------------------|----------------------------------------------|
| Control A.....    | considerable.....                    | 1.56                                         |
| Tests A.....      | much reduced.....                    | 2.16                                         |
| Control B.....    | considerable.....                    | 1.84                                         |
| Tests B.....      | much reduced.....                    | 2.08                                         |

The accompanying drawing further illustrates the present invention. Figures 1, 2 and 3 are sectional views showing a suitable photographic support layer 10 to which is applied the anti-bronzing agent of the present invention. In Figure 1, the support 10, which may be the conventional photographic paper, contains the anti-bronzing agent in the emulsion layer 11. In Figure 2 the support 10 has applied thereto an emulsion layer 12 and a super coat 13 containing the anti-bronzing agent. In Figure 3 the support 10 and the emulsion layer 12 are separated by a sub coat 14 containing the anti-bronzing agent.

What we claim is:

1. A photographic element including a photographic silver halide emulsion layer and in contact therewith and uniformly distributed thereover a heterocyclic compound selected from the class of those represented by the following general formulae:



and



where X is selected from the class consisting of oxygen and sulphur atoms, Y is selected from the class consisting of oxygen and sulphur atoms and imino groups, and D is selected from the class consisting of substituted and unsubstituted carbon atoms completing a six-membered ring.

2. A photographic element as defined in claim 1 in which the heterocyclic compound is 2:5-dimercapto-1:3:4-thiodiazole.

3. A photographic element as defined in claim 1 in which the heterocyclic compound is 2-mercapto-5-amino-1:3:4-thiodiazole.

4. A photographic element as defined in claim 1 in which the heterocyclic compound is 1-mercapto-4-hydroxy-phthalazine.

5. A photographic element as defined in claim

6 in which the heterocyclic compound is 1:4-dimercapto-phthalazine.

6. A photographic element including a photographic silver halide emulsion layer which contains uniformly dispersed therein a heterocyclic compound selected from the class of those represented by the following general formulae:

10



and

15



20

where X is selected from the class consisting of oxygen and sulphur atoms, Y is selected from the class consisting of oxygen and sulphur atoms and imino groups, and D is selected from the class consisting of substituted and unsubstituted carbon atoms completing a six-membered ring.

7. A photographic element as defined in claim 6 in which the heterocyclic compound is 2:5-dimercapto-1:3:4-thiodiazole.

8. A photographic element as defined in claim 6 in which the heterocyclic compound is 2-mercapto-5-amino-1:3:4-thiodiazole.

9. A photographic element as defined in claim 6 in which the heterocyclic compound is 1-mercapto-4-hydroxy-phthalazine.

10. A photographic element as defined in claim 6 in which the heterocyclic compound is 1:4-dimercapto-phthalazine.

11. A photographic element including a photographic silver halide emulsion layer and, adjacent thereto, a water-permeable colloid layer containing uniformly dispersed therein a heterocyclic compound selected from the class of those represented by the following general formulae:

45



and

50



55

55

where X is selected from the class consisting of oxygen and sulphur atoms, Y is selected from the class consisting of oxygen and sulphur atoms and imino groups, and D is selected from the class consisting of substituted and unsubstituted carbon atoms completing a six-membered ring.

12. A photographic element as defined in claim 11 in which the heterocyclic compound is 2:5-dimercapto-1:3:4-thiodiazole.

13. A photographic element as defined in claim 11 in which the heterocyclic compound is 2-mercapto-5-amino-1:3:4-thiodiazole.

14. A photographic element as defined in claim 11 in which the heterocyclic compound is 1-mercapto-4-hydroxy-phthalazine.

15. A photographic element as defined in claim 11 in which the heterocyclic compound is 1:4-dimercapto-phthalazine.

75

16. In a process for improving the quality of a print containing a reduced silver image, the step of hot-glazing said print while in contact with a heterocyclic compound selected from the class of those represented by the following general formulae:



and



where X is selected from the class consisting of oxygen and sulphur atoms, Y is selected from the class consisting of oxygen and sulphur atoms

and imino groups, and D is selected from the class consisting of substituted and unsubstituted carbon atoms completing a six-membered ring.

JOHN DAVID KENDALL,  
DOUGLAS JAMES FRY.

#### REFERENCES CITED

The following references are of record in the file of this patent:

#### UNITED STATES PATENTS

| Number    | Name            | Date          |
|-----------|-----------------|---------------|
| 1,954,334 | Sheppard        | Apr. 10, 1934 |
| 2,099,374 | Schwarz         | Nov. 16, 1937 |
| 2,319,090 | Sheppard et al. | May 11, 1943  |
| 2,353,754 | Peterson        | July 18, 1944 |
| 2,377,375 | Russell         | June 5, 1945  |
| 2,423,767 | Fry             | July 8, 1947  |

#### FOREIGN PATENTS

| Number  | Country       | Date         |
|---------|---------------|--------------|
| 524,556 | Great Britain | Aug. 8, 1940 |